# EUROPEAN PATENT SPECIFICATION

(11) **EP 2 083 437 B1**
(45) Date of publication and mention of the grant of the patent: **28.07.2010**
(21) Application number: 09151084.2
(22) Date of filing: 22.01.2009
(51) Int. Cl.: H01J 17/49, H01J 17/16

(54) **Plasma display panel having high clarity and color purity**
Plasmaanzeigetafel mit hoher Klarheit und Farbreinheit
Panneau d'affichage à plasma

(30) Priority: 23.01.2008 KR 20080007077
(43) Date of publication of application: 29.07.2009
(73) Proprietor: Samsung SDI Co., Ltd., Suwon-si Gyeonggi-do (KR)
(72) Inventor: Yoo, Sung-Hune, Gyeonggi-do (KR)
(74) Representative: Gulde Hengelhaupt Ziebig & Schneider

(56) References cited:
- EP-A- 1 650 782
- US-A1- 2003 102 803

## Description

### Field of the Invention

The present invention relates to a plasma display panel (PDP), and more particularly to, a PDP having a high degree of clarity and color purity obtained by preventing color temperature variance at various viewing angles.

### Description of the Related Art

Plasma display panels (PDPs) may be used for large screen displays, and have good display qualities because of the characteristics of self emission and quick response. PDPs may be formed in a thin configuration, and thus, for example, liquid crystal displays (LCDs) are suitable to be used as wall display devices.

In a PDP, a kind of gas is filled between two electrodes disposed in a sealed space and then a predetermined voltage is applied to the electrodes to cause a glow discharge in the sealed space, therefore, ultraviolet (UV) rays are generated. Phosphor layers, formed in a predetermined pattern, are excited by the generated UV rays and thus emitting visible light to form images.

According to driving methods, PDPs may be classified into direct current (DC)-type PDPs, alternating current (AC)-type PDPs, and hybrid-type PDPs. According to electrode structures, PDPs may also be classified into two-electrode type PDPs and three-electrode type PDPs. DC-type PDPs may include an auxiliary anode inducing an auxiliary discharge, and AC-type PDPs may include address electrodes increasing addressing speed by separately performing a selective discharge and a sustain discharge.

The AC-type PDPs may be further classified into PDPs having an opposing discharge-type electrode structure and PDPs having a surface discharge-type electrode structure, according to arrangements of electrodes. In PDPs having an opposing discharge-type electrode structure, two sustain electrodes which cause a discharge are respectively disposed on a front substrate and a rear substrate and the discharge occurs vertically to the substrates. In PDPs having a surface discharge-type electrode structure, two sustain electrodes which cause a discharge are disposed on the same substrate, and the discharge occurs on a surface of the substrate.

A contemporary PDP may include a front substrate, and sustain electrodes having a predetermined width and a predetermined height formed in pairs on a bottom surface of the front substrate, and each of the pairs of sustain electrodes includes a common electrode and a scan electrode.

A bus electrode to which a voltage is applied is formed on a bottom surface of each of the sustain electrodes. The sustain electrodes and the bus electrodes are covered by a front dielectric layer, and a protective layer is formed on a bottom surface of the front dielectric layer. Such structure is disclosed in US 2003/102803 A1 giving examples of useful materials for the front dielectric layer.

The rear substrate is disposed to face to the front substrate, and address electrodes having a predetermined width and height are formed on the rear substrate. The address electrodes are covered by a rear dielectric layer.

Also, barrier ribs defining discharge spaces and preventing crosstalk between adjacent discharge spaces are formed on the rear dielectric layer. The discharge spaces are filled with the discharge gas, and a phosphor layer formed of red, green, or blue phosphor is formed in each of the discharge spaces.

An AC voltage is applied between a first electrode and a second electrode, for example, a pair of sustain electrodes. When the AC voltage reaches a discharge firing voltage, an electric line of force is generated, thereby dissociating inert gas into electrons and ions. When electrons are recombined with ions, ultraviolet rays (UV) are generated and the phosphor is excited by the generated UV rays, thereby emitting light.

Visible light emitted from a phosphor is sequentially transmitted through the protective layer, which may be formed of MgO, the front dielectric layer, and the front substrate. The orientation of the visible light entering the top panel of the PDP at a predetermined incident angle may be changed according to the refractive index of each layer. For instance, EP 1650782 A2 discloses a plasma display panel, in which the difference in the index of refraction between a dielectric layer and a protective film covering the dielectric layer is taken into consideration. In this regard, the refractive index of each layer changes according to a wavelength of the visible light. That is, the refractive index decreases as the wavelength increases. Therefore, when visible light having different colors incident to the front dielectric layer and the front substrate at a same angle of incidence, blue light is relatively strong when the displayed image is viewed by user located in front of the front substrate (i.e., near to a zero degree angle of incidence). When the user moves to a location away from the zero degree angle of incidence (i.e., a larger angle of incidence), red light becomes stronger, because blue light has a larger refractive index than red light in a same media. Therefore, the color temperature of a PDP may disadvantageously differs in accordance with a viewing angle of the user.

### SUMMARY OF THE INVENTION

It is therefore one object of the present invention to provide an improved PDP in order to overcome the color temperature difference as discussed above.

It is another object of the present invention to provide a PDP having a high degree of clarity and color purity, which is obtained by maintaining constant color temperature at different viewing angles.

According to an aspect of the present invention, there is provided a front dielectric layer for a PDP according to claim 1.

The front dielectric layer may include three or more compounds selected from the group consisting of B₂O₃, SiO₂ PbO, BaO, TiO₂, and Al₂O_{3.}

The front dielectric layer may include three or more compounds selected from the group consisting of from 37 mole% to 43 mole% of B₂O₃, 10 mole% to 60 mole% of SiO₂, 15 mole% to 38 mole% of PbO, 0 mole% to 13 mole% of BaO, 0 mole% to 10 mole% of TiO₂, and 0 mole% to 8 mole% of Al₂O₃. Preferably, the mole percentages of the compounds selected above add up to 100%, i.e. the dielectric layer consists of compounds selected from the group consisting of B₂O₃, SiO₂ PbO, BaO, TiO₂, and Al₂O₃.

The front dielectric layer may include three or more compounds selected from the group consisting of B₂O₃, SiO₂, Bi₂O₃, ZnO, and Al₂O₃.

The front dielectric layer may include three or more compounds selected from the group consisting of 10 mole% to 40 mole% of B₂O_{3,} 0 mole% to 12 mole% of SiO₂, 8 mole% to 13 mole% of Bi₂O₃, 10 mole% to 35 mole% of ZnO, and 4 mole% to 13 mole% of Al₂O₃. Preferably, the mole percentages of the compounds selected above add up to 100%, i.e. the dielectric layer consists of compounds selected from the group consisting of B₂O₃, SiO₂, Bi₂O₃, ZnO, and Al₂O₃.

The front substrate and the front dielectric layer are provided with different refractive indices from each other, wherein preferably [(n₄₅₀/n'₄₅₀)-(n₅₅₀/n'₅₅₀)] is less than 0.01, more preferably less than 0.007, [(n₅₅₀/n'₅₅₀)-(n₆₃₀/n'₆₃₀)] is preferably less than 0.01, more preferably less than 0.007, and [(n₄₅₀/n'₄₅₀)-(n_{630/}n'₆₃₀)] is preferably less than 0.01, more preferably less than 0.007, where n₄₅₀ is the refractive index of the front dielectric layer at a wavelength of 450 nm, n'₄₅₀ is the refractive index of the front substrate at a wavelength of 450 nm, n₅₅₀ is the refractive index of the front dielectric layer at a wavelength of 550 nm, n'₅₅₀ is the refractive index of the front substrate at a wavelength of 550 nm, n₆₃₀ is the refractive index of the front dielectric layer at a wavelength of 630 nm, and n'₆₃₀ is the refractive index of the front substrate at a wavelength of 630 nm.

The front dielectric layer may include three or more compounds selected from the group consisting of B₂O₃, SiO₂, PbO, BaO, TiO₂, and Al₂O₃. The front dielectric layer may include three or more compounds selected from the group consisting of 37 mole% to 43 mole% of B₂O₃, 10 mole% to 60 mole% of SiO₂, 15 mole% to 38 mole% of PbO, 0 mole% to 13 mole% of BaO, 0 mole% to 10 mole% of TiO₂, and 0 mole% to 8 mole% of Al₂O₃.

The front dielectric layer may include three or more compounds selected from the group consisting of B₂O₃, SiO₂, Bi₂O₃, ZnO, and Al₂O₃. The front dielectric layer may include three or more compounds selected from the group consisting of 10 mole% to 40 mole% of B₂O₃, 0 mole% to 12 mole% of SiO₂, 8 mole% to 13 mole% of Bi₂O₃, 10 mole% to 35 mole% of ZnO, and 4 mole% to 13 mole% of Al₂O₃.

Accordingly, a method of manufacturing a plasma display panel (PDP) is provided as defined in claim 7. Preferebly [(n₄₅₀/n'₄₅₀)-(n₅₅₀/n'₅₅₀)] is less than 0.01, more preferably less than 0.007, [(n₅₅₀/n'₅₅₀)-(n₆₃₀/n'₆₃₀)] is preferably less than 0.01, more preferably less than 0.007, and preferably [(n₄₅₀/n'₄₅₀)-(n₆₃₀/n'₆₃₀)] is less than 0.01, more preferably less than 0.007, where n₄₅₀ is a refractive index of the front dielectric layer at a wavelength of 450 nm, n'₄₅₀ is a refractive index of the front substrate at a wavelength of 450 nm, n₅₅₀ is a refractive index of the front dielectric layer at a wavelength of 550 nm, n'₅₅₀ is a refractive index of the front substrate at a wavelength of 550 nm, n₆₃₀ is a refractive index of the front dielectric layer at a wavelength of 630 nm, and n'₆₃₀ is a refractive index of the front substrate at a wavelength of 630 nm. The method further comprises the step of preparing the front substrate by depositing a protective layer on the prepared front dielectric layer; preparing a rear dielectric layer by coating a phosphor slurry on an internal surface of discharge cells; preparing a rear substrate by depositing phosphor layers on the prepared rear dielectric layer; and assembling the prepared rear substrate and the front substrate to face to each other and to be spaced apart from each other, and filling gas into the discharge cells vacuumed.

The front dielectric layer may comprise not less than three compounds selected from a group consisting of B₂O₃, SiO₂, PbO, BaO, TiO₂, and Al₂O₃. The front dielectric layer may comprise three or more compounds selected from the group consisting of from 37 mole% to 43 mole% of B₂O₃, from 10 mole% to 60 mole% of SiO₂, from 15 mole% to 38 mole% of PbO, from 0 mole% to 13 mole% of BaO, from 0 mole% to 10 mole% of TiO₂, and from 0 mole% to 8 mole% of Al₂O₃. Preferably, the mole percentages of the selected compounds above add up to 100%.

Alternatively, the front dielectric layer may comprise three or more compounds selected from a group consisting of B₂O₃, SiO₂, Bi₂O₃, ZnO, and Al₂O₃. The front dielectric layer may comprise three or more compounds selected from the group consisting of from 10 mole% to 40 mole% of B₂O₃, 0 mole% to 12 mole% of SiO₂, 8 mole% to 13 mole% of Bi₂O₃, 10 mole% to 35 mole% of ZnO, and 4 mole% to 13 mole% of Al₂O₃. Preferably, the mole percentages of the selected compounds above add up to 100%.

### BRIEF DESCRIPTION OF THE DRAWINGS

A more complete appreciation of the invention, and many of the attendant advantages thereof, will be readily apparent as the same becomes better understood by reference to the following detailed description when considered in conjunction with the accompanying drawings in which like reference symbols indicate the same or similar components, wherein:

FIG. 1 is a cross-sectional view of a part of a contemporary plasma display panel (PDP);

FIG. 2 is a cross-sectional view illustrating visible light refracted through a top panel of the contemporary PDP illustrated in FIG. 1;

FIG. 3A is a two dimensional graph of the difference between the ratio of refractive indices of front dielectric layers and front substrates of the PDPs constructed as Examples 3, 4 and Comparative Examples 3, 4 at wavelengths of 450 nm and 550 nm with respect to a color temperature difference; and

FIG. 3B is a two dimensional graph of the difference between the ratio of refractive indices of the front dielectric layers and the front substrates of the PDPs constructed as Examples 3, 4 and Comparative Examples 3, 4 at wavelengths of 450 nm and 630 nm with respect to a color temperature difference.

### DETAILED DESCRIPTION OF THE INVENTION

The present invention will now be described more fully with reference to the accompanying drawings, in which exemplary embodiments of the invention are shown.

FIG. 1 is a cross-sectional view of a part of a contemporary plasma display panel (PDP);

Referring to FIG. 1, the contemporary PDP includes a front substrate 14, and sustain electrodes 15 having a predetermined width and a predetermined height formed in pairs on a bottom surface of front substrate 14, wherein each of the pairs of sustain electrodes 15 includes a common electrode and a scan electrode.

A bus electrode to which a voltage is applied is formed on a bottom surface of each of sustain electrodes 15. Sustain electrodes 15 and the bus electrodes are covered by a front dielectric layer 16, and a protective layer 17 is formed on a bottom surface of front dielectric layer 16.

Rear substrate 10 is disposed to face front substrate 14, and address electrodes 11 having a predetermined width and height are formed on rear substrate 10. Address electrodes 11 are covered by a rear dielectric layer 12.

Also, barrier ribs 19 defining discharge spaces and preventing crosstalk between adjacent discharge spaces are formed on rear dielectric layer 12. The discharge spaces are filled with discharge gas, and a phosphor layer 13 formed of red, green, or blue phosphor is formed in each of the discharge spaces.

Then, an AC voltage is applied between a first electrode and a second electrode, for example, a pair of sustain electrodes 15. When the AC voltage reaches a discharge firing voltage, an electric line of force is generated, thereby dissociating an inert gas into electrons and ions. When electrons are recombined with ions 18, ultraviolet rays (UV) are generated and the phosphor is excited by the generated UV rays and thus emitting light 20.

FIG. 2 is a cross-sectional view illustrating visible light refracted through a top panel of the contemporary PDP illustrated in FIG. 1.

Referring to FIGS. 1 and 2, visible light emitted from a phosphor is sequentially transmitted through protective layer 17, which may be formed of MgO, front dielectric layer 16, and front substrate 14. The orientation of the visible light entering the top panel of the PDP at a predetermined incident angle is changed according to the refractive index of each layer. In this regard, the refractive index of each layer changes according to a wavelength of the visible light. That is, the refractive index decreases as the wavelength increases. Therefore, when visible lights having different wavelength incidents front dielectric layer 16 and front substrate 14 at a same incident angle, blue light having relative short wavelength is relatively strong when viewed by the user in front of the front substrate (i.e., at approximately zero degree viewing angle with respect to the vertical line of the front substrate). As the user moves to a location away from the front of the front substrate (i.e., a larger viewing angle with respect to the vertical line of the front substrate), however, the red light becomes stronger, because blue light has a larger refractive index than red light. Thus, the color temperature of a PDP may differ according to a viewing angle.

According to the present invention, in a front dielectric layer for a PDP covering sustain electrodes arranged at predetermined intervals on a front substrate, a difference between the ratio of the refractive index of the front dielectric layer to the refractive index of the front substrate at a first wavelength and the respective ratio at a second wavelength may be 0.01 or less, preferably less than 0.01, more preferably less than 0.007. For example, [(n₄₅₀/n'₄₅₀)-(n₅₅₀/n'₅₅₀)], [(n₅₅₀/n'₅₅₀)-(n₆₃₀/n'₆₃₀)], or [(n₄₅₀/n'₄₅₀)-(n₆₃₀/n'₆₃₀)] may be 0.01 or less, preferably less than 0.01, more preferably less than 0.007, where n₄₅₀ is the refractive index of the front dielectric layer at a wavelength of 450 nm, n'₄₅₀ is the refractive index of the front substrate at a wavelength of 450 nm, n₅₅₀ is the refractive index of the front dielectric layer at a wavelength of 550 nm, n'₅₅₀ is the refractive index of the front substrate at a wavelength of 550 nm, n₆₃₀ is the refractive index of the front dielectric layer at a wavelength of 630 nm, and n'₆₃₀ is the refractive index of the front substrate at a wavelength of 630 nm.

The inventors of the present invention surprisingly identified a relationship between a difference of refractive index ratios and a color temperature difference at an interface between two types of materials (a front substrate for a PDP and a front dielectric layer for a PDP), using one kind of a front substrate and front dielectric layers having different refractive indexes from each other.

As a result, the inventors surprisingly found that the difference between the ratio of refractive indices of the front dielectric layer and the front substrate at two wavelengths, that is, [(n₄₅₀/n'₄₅₀)-(n₅₅₀/n'₅₅₀)], [(n₅₅₀/n'₅₅₀)-(n₆₃₀/n'₆₃₀)], or [(n₄₅₀/n'₄₅₀)-(n₆₃₀/n'₆₃₀)] where n₄₅₀ is the refractive index of the front dielectric layer at 450 nm, n'₄₅₀ is the refractive index of the front substrate at 450 nm, n₅₅₀ is the refractive index of the front dielectric layer at 550 nm, n'₅₅₀ is the refractive index of the front substrate at 550 nm, n₆₃₀ is the refractive index of the front dielectric layer at 630 nm, and n'₆₃₀ is the refractive index of the front substrate at 630 nm, increases approximately linearly as the color temperature difference increases. That is, the difference between the ratio of refractive index of the front dielectric layer to the refractive index of the front substrate at two wavelengths has a linear proportional relationship to the color temperature difference. It is noted that, as the color temperature difference increases, an image may be degraded due to differences in clarity and color purity at different viewing angles, because as the color temperature difference increases, colors are more distinctively distinguished from each other.

That is, as the difference between the ratio of refractive indices of the front dielectric layer and the front substrate at two wavelengths increases, the color temperature difference increases and thus color temperature may vary and a degree of clarity and color purity may be degraded. In other words, as the difference between the ratio of refractive indices of the front dielectric layer and the front substrate at two wavelengths decreases, the color temperature difference is decreased and thus the color temperature becomes uniform and a degree of clarity and color purity can be maintained constant at various viewing angles.

Surprisingly, it was found that if a color temperature difference of a PDP at various viewing angles is greater than 200K, colors may be distinguished from each other and thus a degree of clarity and color purity may be degraded; on the other hand, when the color temperature difference of a PDP at various viewing angles is 200K or less, colors may not be distinguished from each other and thus a degree of clarity and color purity may be maintained constant at various viewing angles. That is, 200 K may be used as a threshold value for determining whether the color temperature is uniform or non-uniform.

Since the difference between the ratio of refractive indices of the front dielectric layer and the front substrate at two wavelengths has a linear proportional relationship with the color temperature difference, a difference between the ratio of refractive indices of the front dielectric layer and the front substrate at two wavelengths corresponds to a specific color temperature difference value may be identified using a graph of the difference between the ratio of refractive indices of the front dielectric layer and the front substrate at two wavelengths with respect to the color temperature difference.

In order to obtain a difference between the ratio of refractive indices of the front dielectric layer and the front substrate at two wavelengths corresponding to a color temperature difference of 200K, a two dimensional graph having an x axis representing a difference between the ratio of refractive indices of the front dielectric layer and the front substrate at two wavelengths and a y axis representing a color temperature difference is obtained. As a result, the difference between the ratio of refractive indices of the front dielectric layer and the front substrate at two wavelengths corresponding to a color temperature difference of 200 K may be 0.01.

In other words, when the difference between the refractive index ratio of the front dielectric layer and the front substrate at the first wavelength and the refractive index ratio of the front dielectric layer and the front substrate at the second wavelength, that is, [(n₄₅₀/n'₄₅₀)-(n₅₅₀/n'₅₅₀)], [(n₅₅₀/n'₅₅₀)-(n₆₃₀/n'₆₃₀)] or [(n₄₅₀/n'₄₅₀)-(n₆₃₀/n'₆₃₀)] is 0.01 or less, preferably less than 0.01, more preferably less than 0.007, the color temperature difference is 200K or less. Therefore, no color separation occurs and a decrease in a degree of clarity and color purity can be hindered.

The front dielectric layer used in the present invention may have any composition such that the difference between the refractive index ratio of the front dielectric layer and the front substrate at the first wavelength and the difference between the refractive index ratio of the front dielectric layer and the front substrate at the second wavelength is 0.01 or less, preferably less than 0.01, more preferably less than 0.007. For example, the front dielectric layer may include three or more compounds selected from B₂O₃, SiO₂, PbO, BaO, TiO₂, and Al₂O_{3.}

Specifically, the front substrate is formed of glass, and the front dielectric layer may include three or more compounds selected from 37 mole% to 43 mole% of B₂O₃, 10 mole% to 60 mole% of SiO₂, 15 mole% to 38 mole% of PbO, 0 mole% to 13 mole% of BaO, 0 mole% to 10 mole% of TiO₂, and 0 mole% to 8 mole% of Al₂O₃. Within such ranges, the difference between the refractive index ratio of the front dielectric layer and the front substrate at the first wavelength and the difference between the refractive index ratio of the front dielectric layer and the front substrate at the second wavelength is 0.01 or less, preferably less than 0.01, more preferably less than 0.007.

In other embodiments, the front dielectric layer may include three or more compounds selected from B₂O₃, SiO₂, Bi₂O₃, ZnO, and Al₂O₃.

Specifically, the front dielectric layer may include three or more compounds selected from 10 mole% to 40 mole% of B₂O₃, 0 mole% to 12 mole% of SiO₂, 8 mole% to 13 mole% of Bi₂O₃, 10 mole% to 35 mole% of ZnO, and 4 mole% to 13 mole% of Al₂O₃. Within such ranges, the difference between the refractive index ratio of the front dielectric layer and the front substrate at the first wavelength and the difference between the refractive index ratio of the front dielectric layer and the front substrate at the second wavelength is 0.01 or less, preferably less than 0.01, more preferably less than 0.007.

A PDP according to an embodiment of the present invention includes a front substrate on which sustain electrodes arranged at predetermined intervals are disposed; a front dielectric layer covering the sustain electrodes; a rear substrate disposed to face the front substrate, on which address electrodes extending in a direction perpendicular to a direction in which the sustain electrodes extend are disposed; a rear dielectric layer covering the address electrodes; barrier ribs defining discharge spaces between the front substrate and the rear substrate; and phosphor layers formed in the discharge spaces, wherein [(n₄₅₀/n'₄₅₀)-(n₅₅₀/n'₅₅₀)], [(n₅₅₀/n'₅₅₀)-(n₆₃₀/n'₆₃₀)] and [(n₄₅₀/n'₄₅₀)-(n₆₃₀/n'₆₃₀)] is 0.01 or less, preferably less than 0.01, more preferably less than 0.007, where n₄₅₀ is the refractive index of the front dielectric layer at 450 nm, n'₄₅₀ is the refractive index of the front substrate at 450 nm, n₅₅₀ is the refractive index of the front dielectric layer at 550 nm, n'₅₅₀ is the refractive index of the front substrate at 550 nm, n₆₃₀ is the refractive index of the front dielectric layer at 630 nm, and n'₆₃₀ is the refractive index of the front substrate at 630 nm.

In the PDP according to the current embodiment, the front dielectric layer may have any composition such that the difference between the refractive index ratio of the front dielectric layer and the front substrate at the first wavelength and the difference between the refractive index ratio of the front dielectric layer and the front substrate at the second wavelength is 0.01 or less, preferably less than 0.01, more preferably less than 0.007.

According to an embodiment of the present invention, the front dielectric layer of the PDP may include three or more compounds selected from B₂O₃, SiO₂, PbO, BaO, TiO₂ and Al₂O₃.

Specifically, the front dielectric layer of the PDP may include three or more compounds selected from 37 mole% to 43 mole% of B₂O₃, 10 mole% to 60 mole% of SiO₂, 15 mole% to 38 mole% of PbO, 0 mole% to 13 mole% of BaO, 0 mole% to 10 mole% of TiO₂, and 0 mole% to 8 mole% of Al₂O₃. Within such ranges, the difference between the refractive index ratio of the front dielectric layer and the front substrate at the first wavelength and the difference between the refractive index ratio of the front dielectric layer and the front substrate at the second wavelength is 0.01 or less, preferably less than 0.01, more preferably less than 0.007.

Alternatively, the front dielectric layer of the PDP may include three or more compounds selected from B₂O₃, SiO₂, Bi₂O₃, ZnO, and Al₂O₃.

Specifically, the front dielectric layer may include three or more compounds selected from 10 mole% to 40 mole% of B₂O₃, 0 mole% to 12 mole% of SiO₂, 8 mole% to 13 mole% of Bi₂O₃, 10 mole% to 35 mole% of ZnO, and 4 mole% to 13 mole% of Al₂O₃. Within such ranges, the difference between the refractive index ratio of the front dielectric layer and the front substrate at the first wavelength and the difference between the refractive index ratio of the front dielectric layer and the front substrate at the second wavelength is 0.01 or less, preferably less than 0.01, more preferably less than 0.007.

The present invention will be described in further details with reference to the following examples of a front dielectric layer for a PDP and a PDP including the front dielectric layer. These examples are for illustrative purposes only and are not intended to limit the scope of the present invention. Those that was not disclosed specifically in the following examples might be performed with any prior art that is known to one of ordinary skill in the art.

### Examples

### Preparation of Dielectric Slurry 1 (Bi-based)

Ethylcellulose that acts as a binder was dissolved in a solvent mixture of butylcarbitolacetate and terpineol in a ratio of 3:7. Then, the resultant mixture was mixed with a glass composition including 13 mole% of Bi₂O₃, 12 mole% of SiO₂, 40 mole% of B₂O₃, and 35 mole% of ZnO to prepare a dielectric slurry 1 having a solid content of 75 %.

### Preparation of Dielectric Slurry 2 (Pb-based)

Ethylcellulose that acts as a binder was dissolved in a solvent mixture of butylcarbitolacetate and terpineol in a ratio of 3:7. Then, the resultant mixture was mixed with a glass composition including 35 mole% of PbO, 40 mole% of B₂O₃, and 25 mole% of SiO₂ to prepare a dielectric slurry 2 having a solid content of 75 %.

### Example 1: Preparation of Front Substrate 1 for PDP

Dielectric slurry 1 was coated on an electrode layer formed on a glass substrate to form a dielectric layer 1 having a thickness of 30µm. Dielectric layer 1 was transparent.

A MgO protective layer was deposited on dielectric layer 1 using a physical vapor deposition (PVD) method, thereby completing the manufacture of a front substrate 1.

### Example 2: Preparation of Front Substrate 2 for PDP

A front substrate 2 was manufactured in the same manner as in Example 1, except that dielectric slurry 2 was used instead of the dielectric slurry 1.

### Preparation of Rear Substrate

6 parts by weight of ethylcellulose that acts as a binder was mixed with 100 parts by weight of a solvent mixture of butylcarbitolacetate and terpineol in a mixture ratio of 3:7. Then, the resultant mixture was mixed with BaMgAl₁₀O₁₇:Eu that acts as a blue phosphor to prepare a phosphor slurry. The obtained phosphor slurry was coated on the inside surface of discharge cells defined by barrier ribs on a first substrate, and then the first substrate having the coated phosphor slurry was dried at 120°C and sintered at 480°C to form a blue phosphor layer.

Also, a (Y,Gd)BO₃:Eu phosphor layer and a ZnSiO₄:Mn phosphor layer were respectively formed in red and green discharge cells in the same manner as described above, thereby completing the manufacture of a rear substrate.

### Example 3: Preparation of PDP 1

The rear substrate and the front substrate 1 were assembled to face each other and form a discharge space, the discharge space was vacuumed, a gas was injected into the discharge space, and then the structure was aged, thereby manufacturing a PDP 1.

### Example 4: Preparation of PDP 2

A PDP 2 was manufactured in the same manner as in Example 3 except that the front substrate 2 was used instead of the front substrate 1.

### Comparative Examples

### Preparation of Dielectric Slurry 3

Ethylcellulose that acts as a binder was dissolved in a solvent mixture of butylcarbitolacetate and terpineol in a ratio of 3:7. Then, the resultant mixture was mixed with a glass composition including 27 mole% of PbO, 43 mole% of B₂O₃, and 30 mole% of BaO to prepare a dielectric slurry 3 having a solid content of 75 %.

### Preparation of Dielectric Slurry 4

Ethylcellulose that acts as a binder was dissolved in a solvent mixture of butylcarbitolacetate and terpineol in a ratio of 3:7. Then, the resultant mixture was mixed with a glass composition including 14 mole% of Bi₂O₃, 52 mole% of B₂O₃, and 34 mole% of ZnO to prepare a dielectric slurry 4 having a solid content of 75 %.

### Comparative Example 1: Preparation of Front Substrate 3 for PDP

A front substrate 3 was prepared in the same manner as in Example 1, except that dielectric slurry 3 was used.

### Comparative Example 2: Preparation of Front Substrate 4 for PDP

A front substrate 4 was prepared in the same manner as in Example 1, except that dielectric slurry 4 was used.

### Comparative Example 3: Preparation of PDP 3

A PDP 3 was manufactured in the same manner as in Example 3, except that front substrate 3 was used.

### Comparative Example 4: Preparation of PDP 4

A PDP 4 was manufactured in the same manner as in Example 3, except that front substrate 4 was used.

The ratios of the refractive indexes of the front substrates 1 through 4 of the PDPs prepared according to Examples 1 and 2 and Comparative Examples 1 and 2 was measured at 450 nm, 550 nm, and 630 nm. The results are shown in Table 1 below.

The refractive indexes were measured using a contemporary refraction measurement method.

**Table 1 Ratio of refractive indexes for examples 1 and 2 with dielectric slurries 1 and 2 and comparative examples 1 and 2 with dielectric slurries 3 and 4**

| Ratio of refractive indexes | Example 1 | Example 2 | Comparative Example 1 | Comparative Example 2 |
|---|---|---|---|---|
| n₄₅₀/n'₄₅₀ | 1.152 | 1.129 | 1.190 | 1.167 |
| n₅₅₀/n'₅₅₀ | 1.147 | 1.125 | 1.178 | 1.158 |
| n₆₃₀/n'₆₃₀ | 1.145 | 1.123 | 1.167 | 1.154 |

Referring to Table 1, n₄₅₀, n₅₅₀, and n₆₃₀ respectively represent the refractive index of the front dielectric layer (dielectric layers 1-4) at 450 nm, 550 nm, and 630 nm, and n'₄₅₀, n'₅₅₀ and n'₆₃₀ respectively represent the refractive index of the front substrate (front substrates 1 through 4) at 450 nm, 550 nm, and 630 nm.

The color temperature of the PDPs 1 through 4 including the front substrates 1 through 4 was measured to identify whether the color temperature is uniform or not. The results are shown in Table 2 below.

Whether the color temperature is uniform or not was able to be identified by measuring the color temperature of an image at various viewing angles and additionally with the naked eye.

Also, the color temperature difference of the PDPs 1 through 4 at 450 nm and 550 nm and the color temperature difference of the PDPs 1 through 4 at 450 nm and 630 nm were measured.

The color temperature difference was measured using a contemporary color temperature measurement device and method.

The relationship between the obtained color temperature difference values and corresponding refractive index ratio difference values is shown in FIGS. 3 and 4. The refractive index ratio differences are shown in Table 2 below. The measured values were rounded to three decimal places and are shown in Tables 1 and 2. Therefore, such data in Table 1 may not precisely correspond to Table 2.

**Table 2 Difference in refractive index ratios for PDP examples 3 and 4 and PDP comparative examples 3 and 4**

| Difference of the refractive index ratios at various wavelengths | Example 3 | Example 4 | Comparative Example 3 | Comparative Example 4 |
|---|---|---|---|---|
| (n₄₅₀/n'₄₅₀)-(n₅₅₀/n'₅₅₀) | 0.004 | 0.004 | 0.011 | 0.009 |
| (n₅₅₀/n'₅₅₀)-(n₆₃₀/n'₆₃₀) | 0.005 | 0.004 | 0.014 | 0.012 |
| (n₄₅₀/n'₄₅₀)-(n₆₃₀/n'₆₃₀) | 0.006 | 0.006 | 0.016 | 0.013 |
| Whether color temperature variance occurs | no | no | yes | yes |

The difference between the ratio of refractive indices of front dielectric layers 1 and 2 and front substrates 1 and 2 of the PDPs 1 and 2 prepared according to Examples 3 and 4 at two wavelengths was 0.01 or less and the color temperature difference was 200 K or less. Color temperature variance did not occur. The difference between the ratio of refractive indices of the front dielectric layers 3 and 4 and the front substrates 3 and 4 of the PDPs 3 and 4 prepared according to Comparative Examples 3 and 4 at two wavelengths was more than 0.01. Color temperature variance occured.

Referring to FIGS. 3A and 3B, it may be seen that the difference between the ratio of refractive indices of the front dielectric layer and the front substrate at two wavelengths corresponding to a color temperature difference of 200K is 0.01. In FIG. 3A, three measurement points are employed according to [(n₄₅₀/n'₄₅₀)-(n₅₅₀/n'₅₅₀)] as shown in Table 2 and the corresponding measured color temperature difference (K). In FIG. 3B, three measurement points are employed according to [(n₄₅₀/n'₄₅₀)-(n₆₃₀/n'₆₃₀)] as shown in Table 2 and the corresponding measured color temperature difference (K).

As described above, a degree of clarity and color purity may be maintained constant by adjusting the difference between the refractive index ratio of a front dielectric layer and a front substrate at two wavelengths selected from 450 nm, 550 nm, and 630 nm to be 0.01 or less, preferably less than 0.01, more preferably less than 0.007.

While the present invention has been particularly shown and described with reference to exemplary embodiments thereof, it will be understood by those of ordinary skill in the art that changes in form and details may be made therein without departing from the scope of the present invention as defined by the following claims.

## Claims

1. A plasma display panel (PDP), comprising:
a front substrate (14), the front substrate (14) having a refractive index (n'₄₅₀) at a, wavelength of 450 nm, a refractive index (n'₅₅₀) at a wavelength of 550 nm, and a refractive index (n'₆₃₀) at a wavelength of 630 nm;
sustain electrodes (15) arranged at predetermined intervals on the front substrate (14);
and
a front dielectric layer (16) covering the sustain electrodes (15) arranged at predetermined intervals on the front substrate (14), the front dielectric layer (16) having a refractive index (n₄₅₀) at a wavelength of 450 nm, a refractive index (n₅₅₀) at a wavelength of 550 nm, and a refractive index (n₆₃₀) at a wavelength of 630 nm;
**characterized in that**
the front substrate (14) and the front dielectric layer (16) have different refractive indices from each other, wherein:
the value of the difference [(n₄₅₀/n'₄₅₀)-(n₅₅₀/n'₅₅₀)], i.e. the difference between the ratio of the refractive indices of the front dielectric layer (16) and the front substrate (14) at 450 nm and at 550 nm, is less or equal to 0.01,
the value of the difference [(n₅₅₀/n'₅₅₀)-(n₆₃₀/n'₆₃₀)], i.e. the difference between the ratio of the refractive indices of the front dielectric layer (16) and the front substrate (14) at 550 nm and at 630 nm, is less or equal to 0.01, and
the value of the difference [(n₄₅₀/n'₄₅₀)-(n₆₃₀/n'₆₃₀)], i.e. the difference between the ratio of the refractive indices of the front dielectric layer (16) and the front substrate (14) at 450 nm and at 630 nm, is less or equal to 0.01.

2. The plasma display panel (PDP) of claim 1, in which the front dielectric layer (16) comprises not less than three compounds selected from a group consisting of B₂O₃, SiO₂, PbO, BaO, TiO₂, and Al₂O₃.

3. The plasma display panel (PDP) of claim 1, in which the front dielectric layer (16) comprises three or more compounds selected from the group consisting of from 37 mole% to 43 mole% of B₂O₃, from 10 mole% to 60 mole% of SiO₂, from 15 mole% to 38 mole% of PbO, from 0 mole% to 13 mole% of BaO, from 0 mole% to 10 mole% of TiO₂ and from 0 mole% to 8 mole% of Al₂O₃.

4. The plasma display panel (PDP) of claim 1, in which the front dielectric layer (16) comprises three or more compounds selected from a group consisting of B₂O₃, SiO₂ Bi₂O₃, ZnO, and Al₂O₃.

5. The plasma display panel (PDP) of claim 1, in which the front dielectric layer (16) comprises three or more compounds selected from the group consisting of from 10 mole% to 40 mole% of B₂O₃, 0 mole% to 12 mole% of SiO₂, 8 mole% to 13 mole% of Bi₂O₃, 10 mole% to 35 mole% of ZnO, and 4 mole% to 13 mole% of Al₂O₃.

6. The plasma display panel (PDP) of any of the previous claims, in which the front substrate (14) is formed of glass.

7. A method of manufacturing a plasma display panel (PDP), the method comprising:
preparing a front dielectric layer (16) by coating a dielectric slurry on an electrode layer formed on a glass substrate, with the front dielectric layer (16) covering sustain electrodes (15) arranged at predetermined intervals on a front substrate (14),;
preparing the front substrate (14) by depositing a protective layer (17) on the prepared front dielectric layer (16);
preparing a rear dielectric layer (12) by coating a phosphor slurry on an internal surface of discharge cells;
preparing a rear substrate (10) by depositing phosphor layers on the prepared rear dielectric layer (12); and
assembling the prepared rear substrate (10) and the front substrate (14) to face each other and to be spaced apart from each other, and filling gas into the discharge cells vacuumed, **characterized in** by
providing the front substrate (14) and the front dielectric layer (16) with different refractive indices from each other such that [(n₄₅₀/n'₄₅₀)-(n₅₅₀/n'₅₅₀)] is not more than 0.01, [(n₅₅₀/n'₅₅₀)-(n₆₃₀/n'₆₃₀)] is not more than 0.01, and [(n₄₅₀/n'₄₅₀)-(n₆₃₀/n'₆₃₀)] is not more than 0.01, where n₄₅₀ is a refractive index of the front dielectric layer (16) at a wavelength of 450 nm, n'₄₅₀ is a refractive index of the front substrate (14) at a wavelength of 450 nm, n₅₅₀ is a refractive index of the front dielectric layer (16) at a wavelength of 550 nm, n'₅₅₀ is a refractive index of the front substrate (14) at a wavelength of 550 nm, n₆₃₀ is a refractive index of the front dielectric layer (16) at a wavelength of 630 nm, and n'₆₃₀ is a refractive index of the front substrate (14) at a wavelength of 630 nm.

8. The method of claim 7, in which the front dielectric layer (16) comprises not less than three compounds selected from a group consisting of B₂O₃, SiO₂, PbO, BaO, TiO₂ and Al₂O₃.

9. The method of claim 7, in which the front dielectric layer (16) comprises three or more compounds selected from the group consisting of from 37 mole% to 43 mole% of B₂O₃, from 10 mole% to 60 mole% of SiO₂, from 15 mole% to 38 mole% of PbO, from 0 mole% to 13 mole% of BaO, from 0 mole% to 10 mole% of TiO₂, and from 0 mole% to 8 mole% of Al₂O₃.

10. The method of claim 7, in which the front dielectric layer (16) comprises three or more compounds selected from a group consisting of B₂O₃, SiO₂ Bi₂O₃, ZnO, and Al₂O₃.

11. The method of claim 7, in which the front dielectric layer (16) comprises three or more compounds selected from the group consisting of from 10 mole% to 40 mole% of B₂O₃, 0 mole% to 12 mole% of SiO₂, 8 mole% to 13 mole% of Bi₂O₃, 10 mole% to 35 mole% of ZnO, and 4 mole% to 13 mole% of Al₂O₃.

12. The method of any of the previous claims 7 to 11, in which the front substrate (14) is formed of glass.

## Patentansprüche

1. Plasmaanzeigetafel (PDP), aufweisend:
ein vorderes Substrat (14), wobei das vordere Substrat (14) einen Brechungsindex (n'₄₅₀) bei einer Wellenlänge von 450 nm, einen Brechungsindex (n'₅₅₀) bei einer Wellenlänge von 550 nm und einen Brechungsindex (n'₆₃₀) bei einer Wellenlänge von 630 nm aufweist;
Sustain-Elektroden (15), die in vorbestimmten Abständen auf dem vorderen Substrat (14) angeordnet sind; und
eine vordere dielektrische Schicht (16), die die in vorbestimmten Abständen auf dem vorderen Substrat (14) angeordneten Sustain-Elektroden (15) bedeckt, wobei die vordere dielektrische Schicht (16) einen Brechungsindex (n₄₅₀) bei einer Wellenlänge von 450 nm, einen Brechungsindex (n₅₅₀) bei einer Wellenlänge von 550 nm und einen Brechungsindex (n₆₃₀) bei einer Wellenlänge von 630 nm aufweist;
**dadurch gekennzeichnet, dass**
das vordere Substrat (14) und die vordere dielektrische Schicht (16) Brechungsindices aufweisen, die sich voneinander unterscheiden, wobei:
der Wert der Differenz [(n₄₅₀/n'₄₅₀)-(n₅₅₀/n'₅₅₀)], d.h., der Differenz zwischen dem Verhältnis der Brechungsindices der vorderen dielektrischen Schicht (16) und des vorderen Substrats (14) bei 450 nm und bei 550 nm kleiner/gleich 0,01 ist,
der Wert der Differenz [(n₅₅₀/n'₅₅₀)-(n₆₃₀/n'₆₃₀)], d.h., der Differenz zwischen dem Verhältnis der Brechungsindices der vorderen dielektrischen Schicht (16) und des vorderen Substrats (14) bei 550 nm und bei 630 nm kleiner/gleich 0,01 ist, und
der Wert der Differenz [(n₄₅₀/n'₄₅₀)-(n₆₃₀/n'₆₃₀)], d.h., der Differenz zwischen dem Verhältnis der Brechungsindices der vorderen dielektrischen Schicht (16) und des vorderen Substrats (14) bei 450 nm und bei 630 nm kleiner/gleich 0,01 ist.

2. Plasmaanzeigetafel (PDP) nach Anspruch 1, wobei die vordere dielektrische Schicht (16) nicht weniger als drei Verbindungen aufweist, die aus einer Gruppe bestehend aus B₂O₃, SiO₂, PbO, BaO, TiO₂ und Al₂O₃ ausgewählt sind.

3. Plasmaanzeigetafel (PDP) nach Anspruch 1, wobei die vordere dielektrische Schicht (16) drei oder mehr Verbindungen aufweist, die aus der Gruppe bestehend aus 37 Mol-% bis 43 Mol-% B₂O₃, 10 Mol-% bis 60 Mol-% SiO₂, 15 Mol-% bis 38 Mol-% PbO, 0 Mol-% bis 13 Mol-% BaO, 0 Mol-% bis 10 Mol-% TiO₂ und 0 Mol-% bis 8 Mol-% Al₂O₃ ausgewählt sind.

4. Plasmaanzeigetafel (PDP) nach Anspruch 1, wobei die vordere dielektrische Schicht (16) drei oder mehr Verbindungen aufweist, die aus einer Gruppe bestehend aus B₂O₃, SiO₂, Bi₂O₃, ZnO und Al₂O₃ ausgewählt sind.

5. Plasmaanzeigetafel (PDP) nach Anspruch 1, wobei die vordere dielektrische Schicht (16) drei oder mehr Verbindungen aufweist, die aus der Gruppe bestehend aus 10 Mol-% bis 40 Mol-% B₂O₃, 0 Mol-% bis 12 Mol-% SiO₂, 8 Mol-% bis 13 Mol-% Bi₂O₃, 10 Mol-% bis 35 Mol-% ZnO und 4 Mol-% bis 13 Mol-% Al₂O₃ ausgewählt sind.

6. Plasmaanzeigetafel (PDP) nach einem der vorhergehenden Ansprüche wobei das vordere Substrat (14) aus Glas ausgebildet ist.

7. Verfahren zur Herstellung einer Plasmaanzeigetafel (PDP), wobei das Verfahren aufweist:
Herstellung einer vorderen dielektrischen Schicht (16) durch Aufbringen einer wässrigen dielektrischen Masse auf einer Elektrodenschicht, die auf einem Glassubstrat ausgebildet ist, wobei die vordere dielektrische Schicht (16) Sustain-Elektroden (15) bedeckt, die in vorbestimmten Abständen auf einem vorderen Substrat (14) angeordnet sind;
Herstellen des vorderen Substrats (14) durch Abscheidung einer Schutzschicht (17) auf der hergestellten vorderen dielektrischen Schicht (16);
Herstellen einer hinteren dielektrischen Schicht (12) durch Aufbringen einer wässrigen Phosphormasse auf einer Innenoberfläche von Entladungszellen;
Herstellen eines hinteren Substrats (10) durch Abscheidung von Phosphorschichten auf der hergestellten hinteren dielektrischen Schicht (12); und
Zusammenfügen des hergestellten hinteren Substrats (10) und des hergestellten vorderen Substrats (14) derart, dass sie einander zugewandt und voneinander beabstandet sind, und Füllen von Gas in die vakuumierten Entladungszellen,
**gekennzeichnet durch**
das Bereitstellen des vorderen Substrats (14) und der vorderen dielektrischen Schicht (16) mit Brechungsindices, die sich derart voneinander unterscheiden, dass [(n₄₅₀/n'₄₅₀)-(n₅₅₀/n'₅₅₀)] nicht größer als 0,01 ist, dass [(n₅₅₀/n'₅₅₀)-(n₆₃₀/n'₆₃₀)] nicht größer als 0,01 ist, und dass [(n₄₅₀/n'₄₅₀)-(n₆₃₀/n'₆₃₀)] nicht größer als 0,01 ist, wobei n₄₅₀ ein Brechungsindex der vorderen dielektrischen Schicht (16) bei einer Wellenlänge von 450 nm ist, n'₄₅₀ ein Brechungsindex des vorderen Substrats (14) bei einer Wellenlänge von 450 nm ist, n₅₅₀ ein Brechungsindex der vorderen dielektrischen Schicht (16) bei einer Wellenlänge von 550 nm ist, n'₅₅₀ ein Brechungsindex des vorderen Substrats (14) bei einer Wellelänge von 550 nm ist, n₆₃₀ ein Brechungsindex der vorderen dielektrischen Schicht (16) bei einer Wellenlänge von 630 nm ist, und n'₆₃₀ ein Brechungsindex des vorderen Substrats (14) bei einer Wellenlänge von 630 nm ist.

8. Verfahren nach Anspruch 7, wobei die vordere dielektrische Schicht (16) nicht weniger als drei Verbindungen aufweist, die aus einer Gruppe bestehend aus B₂O₃, SiO₂, PbO, BaO, TiO₂ und Al₂O₃ ausgewählt sind.

9. Verfahren nach Anspruch 7, wobei die vordere dielektrische Schicht (16) drei oder mehr Verbindungen aufweist, die aus der Gruppe bestehend aus 37 Mol-% bis 43 Mol-% B₂O₃, 10 Mol-% bis 60 Mol-% SiO₂, 15 Mol-% bis 38 Mol-% PbO, 0 Mol-% bis 13 Mol-% BaO, 0 Mol-% bis 10 Mol-% TiO₂ und 0 Mol-% bis 8 Mol-% Al₂O₃ ausgewählt sind.

10. Verfahren nach Anspruch 7, wobei die vordere dielektrische Schicht (16) drei oder mehr Verbindungen aufweist, die aus einer Gruppe bestehend aus B₂O₃, SiO₂, Bi₂O₃, ZnO und Al₂O₃ ausgewählt sind.

11. Verfahren nach Anspruch 7, wobei die vordere dielektrische Schicht (16) drei oder mehr Verbindungen aufweist, die aus der Gruppe bestehend aus 10 Mol-% bis 40 Mol-% B₂O₃, 0 Mol-% bis 12 Mol-% SiO₂, 8 Mol-% bis 13 Mol-% Bi₂O₃, 10 Mol-% bis 35 Mol-% ZnO und 4 Mol-% bis 13 Mol-% Al₂O₃ ausgewählt sind.

12. Verfahren nach einem der vorhergehenden Ansprüche 7 bis 11, wobei das vordere Substrat (14) aus Glas ausgebildet ist.

## Revendications

1. Panneau d'affichage à plasma (PDP), comprenant :
un substrat de face (14), le substrat de face (14) ayant un indice de réfraction (n' ₄₅₀) à une longueur d'onde de 450 nm, un indice de réfraction (n'₅₅₀) à une longueur d'onde de 550 nm et un indice de réfraction (n'₆₃₀) à une longueur d'onde de 630 nm ;
des électrodes de maintien (15) agencées à intervalles prédéterminés sur le substrat de face (14) ; et
une couche diélectrique de face (16) couvrant les électrodes de maintien (15) agencées à intervalles prédéterminés sur le substrat de face (14), la couche diélectrique de face (16) ayant un indice de réfraction (n₄₅₀) à une longueur d'onde de 450 nm, un indice de réfraction (n₅₅₀) à une longueur d'onde de 550 nm et un indice de réfraction (n₆₃₀) à une longueur d'onde de 630 nm ;
**caractérisé en ce que**
le substrat de face (14) et la couche diélectrique de face (16) ont des indices de réfraction différents, où
la valeur de la différence [(n₄₅₀/n'₄₅₀)-(n₅₅₀/n'₅₅₀)], c'est à dire la différence entre le rapport des indices de réfraction de la couche diélectrique de face (16) et du substrat de face (14) à 450 nm et à 550 nm, est inférieure ou égale à 0,01,
la valeur de la différence [(n₅₅₀/n'₅₅₀)-(n₃₆₀/n'₃₆₀)], c'est à dire la différence entre le rapport des indices de réfraction de la couche diélectrique de face (16) et du substrat de face (14) à 550 nm et à 630 nm, est inférieure ou égale à 0,01, et
la valeur de la différence [(n₄₅₀/n'₄₅₀)-(n₆₃₀/n'₆₃₀)], c'est-à-dire la différence entre le rapport des indices de réfraction de la couche diélectrique de face (16) et du substrat de face (14) à 450 nm et à 630 nm, est inférieure ou égale à 0,01.

2. Panneau d'affichage à plasma (PDP) de la revendication 1, dans lequel la couche diélectrique de face (16) comprend pas moins de trois composants, choisis dans le groupe constitué de B₂O₃, de SᵢO₂, de PbO, de BaO, de TᵢO₂, et d'Al₂O₃,

3. Panneau d'affichage à plasma (PDP) de la revendication 1, dans lequel la couche diélectrique de face (16) comprend trois composants ou plus, choisis dans le groupe constitué de 37 % molaire à 43 % molaire de B₂O₃, de 10 % molaire à 60 % molaire de SiO₂, de 15 % molaire à 38 % molaire de PbO, de 0 % molaire à 13 % molaire de BaO, de 0 % molaire à 10 % molaire de TiO₂ et de 0 % molaire à 8 % molaire d'Al₂O₃.

4. Panneau d'affichage à plasma (PDP) de la revendication 1, dans lequel la couche diélectrique de face (16) comprend trois composants ou plus, choisis dans le groupe constitué de B₂O₃, de SᵢO₂, de Bi₂O₃, de ZnO et d'Al₂O₃.

5. Panneau d'affichage à plasma (PDP) de la revendication 1, dans lequel la couche diélectrique de face (16) comprend trois composants ou plus, choisis dans le groupe constitué de 10 % molaire à 40 % molaire de B₂O₃, de 0 % molaire à 12 % molaire de SiO₂, de 8 % molaire à 13 % molaire de Bi₂O₃, de 10 % molaire à 35 % molaire de ZnO et de 4 % molaire à 13 % molaire d'Al₂O₃.

6. Panneau d'affichage à plasma (PDP) de l'une des revendications précédentes, dans lequel le substrat de face (14) est formé de verre.

7. Procédé de fabrication d'un panneau d'affichage à plasma (PDP), le procédé comprenant le fait :
de préparer une couche diélectrique de face (16) en enrobant une boue diélectrique sur une couche d'électrode formée sur un substrat de verre, la couche diélectrique de face (16) couvrant des électrodes de maintien (15) agencées à intervalles prédéterminés sur un substrat de face (14),
de préparer le substrat de face (14) en déposant une couche protectrice (17) sur la couche diélectrique de face (16) préparée ;
de préparer une couche diélectrique de dos (12) en enrobant une boue au phosphore sur une surface interne de cellules de décharge ;
de préparer un substrat de dos (10) en déposant des couches de phosphore sur la couche diélectrique de dos (12) préparée ; et
d'assembler le substrat de dos (10) et le substrat de face (14) préparés de manière à ce qu'ils soient en vis-à-vis et à être espacés l'un de l'autre, et remplir du gaz dans les cellules de décharge sous vide,
**caractérisé par** le fait
de doter le substrat de face (14) et la couche diélectrique de face (16) de différents indices de réfraction de sorte que [(n₄₅₀/n'₄₅₀)-(n₅₅₀/n'₅₅₀)] ne dépasse pas 0,01, [(n₅₅₀/n'₅₅₀)-(n₆₃₀/n'₆₃₀)] ne dépasse pas 0,01, et [(n₄₅₀/n'₄₅₀)-(n₆₃₀/n'₆₃₀)] ne dépasse pas 0,01, où n₄₅₀ est un indice de réfraction de la couche diélectrique de face (16) à une longueur d'onde de 450 nm, n'₄₅₀ est un indice de réfraction du substrat de face (14) à une longueur d'onde de 450 nm, n₅₅₀ est un indice de réfraction de la couche diélectrique de face (16) à une longueur d'onde de 550 nm, n'₅₅₀ est un indice de réfraction du substrat de face (14) à une longueur d'onde de 550 nm, n₆₃₀ est un indice de réfraction de la couche diélectrique de face (16) à une longueur d'onde de 630 nm, et n'₆₃₀ est un indice de réfraction du substrat de face (14) à une longueur d'onde de 630 nm.

8. Procédé de la revendication 7, dans lequel la couche diélectrique de face (16) comprend pas moins de trois composants, choisis dans le groupe constitué de B₂O₃, de SiO₂, de PbO, de BaO, de TᵢO₂ et d'Al₂O₃.

9. Procédé de la revendication 7, dans lequel la couche diélectrique de face (16) comprend trois composants ou plus, choisis dans le groupe constitué de 37 % molaire à 43 % molaire de B₂O₃, de 10 % molaire à 60 % molaire de SiO₂, de 15 % molaire à 38 % molaire de PbO, de 0 % molaire à 13 % molaire de BaO, et de 0 % molaire à 10 % molaire de TiO₂, et de 0 % molaire à 8 % molaire d'Al₂O₃.

10. Procédé de la revendication 7, dans lequel la couche diélectrique de face (16) comprend trois composants ou plus, choisis dans le groupe constitué de B₂O₃, de SiO₂, de Bi₂O₃, de ZnO et d'Al₂O₃.

11. Procédé de la revendication 7, dans lequel la couche diélectrique de face (16) comprend trois composants ou plus, choisis dans le groupe constitué de 10 % molaire à 40 % molaire de B₂O₃, de 0 % molaire à 12 % molaire de SiO₂, de 8 % molaire à 13 % molaire de Bi₂O₃, de 10 % molaire à 35 % molaire de ZnO et de 4 % molaire à 13 % molaire d'Al₂O₃.

12. Procédé de l'une des revendications précédentes 7 à 11, dans lequel le substrat de face (14) est formé de verre.
